

1

2,908,648

## CORROSION-INHIBITED COMPOSITIONS CONTAINING N-(ALKYLARYLSULFONYL) AMINO ACIDS AND SALTS THEREOF

John D. Spivack and Janet B. Peterson, Cranston, and Harry Kroll, Warwick, R.I., assignors to Geigy Chemical Corporation, New York, N.Y., a corporation of Delaware

No Drawing. Application October 21, 1954  
Serial No. 463,842

12 Claims. (Cl. 252—47.5)

This invention relates to compositions having corrosion-inhibited, and especially rust-inhibited properties, which contain alkylarylsulfonyl derivatives. More particularly the present invention relates to organic compositions, especially oleaginous compositions containing an alkylarylsulfonyl derivative, which compositions have the property of preventing or inhibiting corrosion and/or rusting, especially in systems employing water or steam or which may be contaminated with water or steam.

In various equipment in which water and/or steam is used, or which may become contaminated with water or steam during service or storage, corrosion and/or rusting of the metal parts, particularly the ferrous metal parts, is encountered causing material damage to such equipment. The prevention of rust formation is particularly important in the protection of metal surfaces where such surfaces are to be lubricated in the presence of moisture. Moisture may enter lubricating systems of land or marine turbines, for example, by leakage through steam glands and through water-cooled heat exchangers or by condensation from the atmosphere. The presence of rust is injurious because it causes excessive wear of gears and bearing surfaces and may also clog the hydraulic governor system, leading to dangerous operating speeds. Furthermore, the presence of rust has been shown to increase the rate of oxidative breakdown of the lubricant itself.

The present invention is also applicable to anti-rust or slushing compositions employed for the protection of metals against atmospheric corrosion and/or rusting. Such compositions are applied to metallic articles, including fabricated metallic articles and finished or semi-finished metal stock to be stored or for shipment by rail or water, to prevent rusting and/or corrosion thereof. The aim in the use of protective or slushing compositions is to protect objects against attack by moisture by coating them.

Important industrial applications of the corrosion and/or rust preventing compounds of the present invention vary over a wide range. They afford excellent protection when incorporated into the following lubricating oils and dielectric oils: motor oils, diesel oils, aviation engine oils, marine engine lubricants, gear oils, oil field machinery lubricants, ice-machine oils, steam cylinder lubricants, transmission oils, soluble oils, textile oils, cutting oils both soluble containing water and the straight oils, turbine oils, insulating oils; lubricating greases; stable gel-like or solid dispersions of metal soaps in hydrocarbon oils; protective coatings; preservative compounds, slushing oils and greases in which part or all of the hydrocarbon oil may be replaced by metal soaps and other constituents; flushing oils. These have vehicles which would be classed in whole or part as oleaginous.

The alkylarylsulfonyl amino acids and their salts of

2

this invention may be added to a wide variety of vehicles to produce compositions having corrosion-inhibited properties, including acidic aqueous liquids, such as used in metal pickling solutions, to aqueous alcoholic solutions both of the lower monohydric alcohol type and the polyhydric alcohol type, which solutions comprise the commonly employed automobile radiator anti-freeze liquids.

A great many materials have been proposed as coating compositions or as additives to lubricating oils for the prevention of rust formation. In U.S. Letters Patent No. 2,578,725 it is proposed to add various alkanesulfonamidoalkane carboxylic acids of the general formula  $R_1SO_2-NH-R_2COOR_3$  (wherein  $R_1$  is a saturated hydrocarbon of  $C_{12}-C_{20}$ ,  $R_2$  is either aliphatic  $C_{n}H_{2n+1}$  or aryl or aromatic radicals and  $R_3$  is H or an alkali metal or ammonium) to alcohols, ketones and mixtures thereof. The alkanesulfonamidoalkane carboxylic acids used for that purpose are described in U.S. Patent No. 2,225,960 granted December 24, 1940. A specific example is hexadecanesulfonamidoacetic acid of the formula:



The compounds which we utilize as potent corrosive and/or rust inhibiting agents according to the present invention are broadly alkylarylsulfonyl derivatives of an amino acid. The sulfonyl group is attached directly to the aromatic nucleus. Those which are suitable for our purpose are alkylarylsulfonyl amino acids having the empirical formula:



wherein R represents one or two alkyl groups of 8-24 carbon atoms inclusive; Ar represents an aryl group which may be phenyl, naphthyl, anthracyl, phenanthryl, chrysyl (Beilstein, vol. V, p. 718), etc.;  $R_1$  represents a substituent selected from the group consisting of hydrogen, alkyl, hydroxyl, carboxyalkyl and phenyl;  $R_2$  represents a substituent selected from the group consisting of hydrogen, alkyl and carboxyalkyl;  $n$  represents 0, 1 or 2; Y represents hydrogen or a salt forming group. The above type compounds are added to a liquid or semi-solid vehicle in a quantity sufficient to confer corrosion and/or rust prevention to the composition which otherwise tends to permit corrosion of metal when brought in surface contact therewith.

More particularly and important we have found that the corrosive effect of lubricating oils and greases (oleaginous vehicle) upon bearing surfaces, gears and other metallic parts in the presence of water or steam, may be prevented by the incorporation in said oleaginous vehicle of a small amount of a class of compounds which are alkylarylsulfonyl derivatives of amino acids, whose empirical formula has been given in the preceding paragraph. Such compounds, when used in small amounts in oleaginous vehicles, it has been determined by scientifically acceptable tests and by other means, effectively prevent the rusting of metal surfaces, particularly those of ferrous metal, upon exposure to water or steam. These additives, moreover, prevent rusting without influencing other properties of the lubricant disadvantageously.

The members of this class of corrosion preventative agents may be regarded as derivatives of the natural or synthetic amino acids, for example, of glycine, whose structural formula is  $NH_2CH_2COOH$ ,  $\alpha$  and  $\beta$  alanine,

the structural formula of which are  $\text{CH}_3\text{CH}(\text{NH}_2)\text{COOH}$  and  $\text{CH}_2(\text{NH}_2)\text{CH}_2\text{COOH}$  respectively, sarcosine or methyl glycocoll, whose structural formula is



iminodiacetic acid, whose structural formula is



aspartic acid whose structural formula is



glutamic acid whose structural formula is



Non-limiting examples of the new type of compounds which are useful as rust and/or corrosion preventives are: N-(dodecylbenzenesulfonyl) glycine, N-(dodecylbenzenesulfonyl) sarcosine, N-(dodecylbenzenesulfonyl) iminodiacetic acid, N-(dodecylbenzenesulfonyl) glutamic acid, N-(dodecylbenzenesulfonyl) alanine, N-(dinonylnaphthalenesulfonyl) glycine, N-(dinonylnaphthalenesulfonyl) sarcosine, N-(dinonylnaphthalenesulfonyl)-iminodiacetic acid, N-(dinonylnaphthalenesulfonyl) glutamic acid, N-(dinonylnaphthalenesulfonyl) alanine, N-(octadecyl antracenesulfonyl)-sarcosine, N-(octyl xylyl) sarcosine and the like.

The sulfonylated amino acids of the general type of the corrosion preventative agents of our invention can be prepared in a number of ways, for example, as outlined in Equations A, B, C and D below:



The reactants in the process of manufacture may be relatively pure single compounds, for example, pure alkylarylsulfonyl chloride or the sulfonyl amide (see empirical formula of respective first mentioned reactant in Equations A and D), and pure amino acid salt, ester,

or nitrile conforming to the second respective reactant in the empirical formula set forth in equations of processes (A), (B) and (C), and the pure chlorocarboxylic acid salt which is the second reactant in the process of equation D. Or the reactants may be mixtures resulting in a product consisting of a mixture of compounds, all represented by the formula



the symbols in which are defined above.

In further explanation, it may be stated that the R-Ar grouping set forth above may be derived from straight-chain or branched-chain octyl, decyl, dodecyl, tetradecyl, hexadecyl, or octadecyl derivatives of either benzene, naphthalene, anthracene or chrysene or from mixtures thereof. The R-Ar grouping may also be derived from the reduction of fatty acylated or alkenylated aromatic compounds. The products obtained by processes (B) and (C) outlined above may also have more or less unsaponified ester or nitrile groupings present therein in addition to free carboxyl groups or salts thereof.

One of the major uses of the additives of the present invention is in the industrial field of lubrication of metal surfaces employing both oils and greases. Another use is the protection of metals, such as iron or broader the ferrous type metal, in humid atmospheres by preservative oils and slushing oils or greases. The members of the class of compounds of this invention can be used alone in an oleaginous vehicle or solvent. Used thus these additives which function as corrosion inhibitors, may be used in a variety of physical states, e.g., as a dispersion, emulsion or solution. When employed in an oleaginous vehicle, the compounds should be soluble, miscible or dispersible in said vehicle. It should be noted that the term "oleaginous vehicle" is employed in the broader sense and to include hydrocarbon oils, fatty oils, fats, the synthetic lubricants such as those of the polyester, polysiloxane, polyalkylene glycols and polyolefine types, and rustproof bases, etc., which may be used as the medium of application of rust-preventive additive to the metal surface.

The N-(alkylarylsulfonyl) amino acids may be incorporated in the oleaginous vehicle in varying proportions being governed by specific use to which the rust preventive composition is to be put, the degree of rust prevention desired, as well as economic considerations, and on the specific alkylarylsulfonyl amino acid selected. Generally it is sufficient to use an amount between 0.005 and 10% by weight, although greater or lesser amounts may be used.

As indicated supra, the general type of alkylarylsulfonyl amino acids and their salts, which are the corrosion inhibitors of the present inventors, are believed to have been first prepared by the present inventors. For that reason the synthesis of several of these additives by various modes will be described in detail in the subsequent examples which appear in order of arrangement before the rust tests and emulsion tests.

## 60 EXAMPLES OF OUR CORROSION INHIBITORS

*Example 1 of corrosion inhibitor—  
N-(n-dodecylbenzenesulfonyl) sarcosine*

### (A) AND (B) PREPARATION OF N-DODECYL BENZENESULFONYL CHLORIDE

Seventy-four grams (74 g.) (0.30 mole) of n-dodecylbenzene ( $N_d^{25} = 1.483$ , boiling at 4.2 mm. Hg pressure at 165-170° C.) was dissolved in 200 milliliters of methylene chloride in a 1-liter flask fitted with a mechanical stirrer, an air condenser, thermometer and dropping funnel; the entire apparatus was protected from moisture by calcium chloride drying tubes on the condenser and the dropping funnel. The solution was cooled to 10° C. by an external bath. Chlorsulfonic acid (73 g.) (0.63 mole) was added thereto over a period of 35 to 40

minutes while its temperature was kept at  $-10^{\circ}$  C. to  $-7^{\circ}$  C. The reaction mixture became dark brown in color. It was stirred and additional two hours while maintaining its temperature at  $0^{\circ}$  C., followed by two more hours at  $20^{\circ}$  C., whereupon it was let stand at room temperature overnight, i.e., for about fifteen hours. The reaction mixture was poured into 300 grams of ice, and 300 milliliters of diethyl ether were added, intimately mixed therewith, whereupon after stratification the water layer was separated from the upper or ether layer. The water layer was extracted with an additional 300 milliliters of ether. The combined ether extracts were extracted with 300 milliliters of a 5% aqueous solution of sodium bicarbonate also containing 10% by weight of sodium chloride to remove residual inorganic acids. The ether in the purified ether layer was removed by distillation at atmospheric pressure followed by reduced pressure. The residue was taken up in 500 milliliters of acetone and filtered free of inorganic salts. Analysis of the residue (A) from the acetone distillation indicated that product (A) contained about 8.3% of n-dodecylbenzene-sulfonyl chloride, the remainder being n-dodecylbenzene sulfonic acid.

Phosphorus pentachloride (19.3 grams) was added gradually with occasional shaking to product (A) amounting to 28 grams, in an Erlenmeyer flask fitted with a drying tube. After effervescence stopped, the reaction mixture was warmed on a water bath for about 30 minutes. The product was then poured into ice, and extracted with 200 milliliters of ether. The ether extract was thereupon washed with water and then dried over anhydrous sodium sulfate. After being separated, ether was removed by evaporation. The residue, which was product (B), was a viscous, reddish oil, the analysis of which indicated that it consisted of 96%-97% of n-dodecylbenzenesulfonyl chloride.

(C) PREPARATION OF N-(n-DODECYLBENZENESULFONYL) SARCOsINE FROM PRODUCT (B) SUPRA.

Sarcosine (3.6 grams) (0.041 mole) was dissolved in 41 milliliters of 1.0 N solution of sodium hydroxide in water to form its sodium salt, and cooled to  $15^{\circ}$  C. A dioxane solution on n-dodecylbenzenesulfonyl chloride (14.0 grams of product (B) described above dissolved in 50 milliliters of dioxane) and 41 milliliters of 1.0 N aqueous sodium hydroxide were added dropwise simultaneously to the aqueous sarcosine solution of the sodium salt of sarcosine over a period of 20 minutes. The reaction mixture was stirred an additional two hours at room temperature; this contained the sodium salt of N-(n-dodecylbenzenesulfonyl) sarcosine with by-products of the reaction. It was then made acid to pH 2 with 6 N aqueous hydrochloric acid, after which it was extracted with ether. This extract was heated to distill off the ether. The residue (12.8 grams) was crystallized from n-hexane, and there was obtained a white crystalline product melting at  $110-111^{\circ}$  C. (uncorrected). The crystalline product was substantially pure N-(n-dodecylbenzenesulfonyl) sarcosine having a neutralization equivalent weight of 400. The calculated neutralization equivalent weight for N-(n-dodecylbenzenesulfonyl) sarcosine is 397.

Example 2 of corrosion inhibitor—N-(n-dodecylbenzenesulfonyl) iminodiacetic acid

Dimethyl iminodiacetate hydrochloride (7.7 grams) (0.039 mole) was dissolved in 100 milliliters of chloroform contained in a 300 milliliter capacity flask which was fitted with a condenser, stirrer and dropping funnel suitably fitted with calcium chloride drying tubes to protect the reaction mixture from moisture. Triethylamine (8.2 grams) (0.082 mole) was added all at once, and the reaction mixture cooled to room temperature. A dioxane solution of n-dodecylbenzenesulfonyl chloride (14 grams) (0.041 mole) dissolved in 50 milliliters of

dioxane was added dropwise to the reaction mixture while undergoing stirring, over a period of 25 minutes, and this mixture was stirred at room temperature for an hour; it was then heated at reflux for an additional hour.

- 5 The chloroform solution of the reaction product was washed successively with water and 5% aqueous sodium chloride solution, and then dried over anhydrous sodium sulfate. It was then decanted from the drying agent. The residue, after evaporation of chloroform was heated 10 on a steam bath with 100 milliliters of 1 N sodium hydroxide solution in water for two hours. The product was the sodium salt of N-(n-dodecylbenzenesulfonyl) iminodiacetic acid in solution. The alkaline solution was extracted with 100 milliliters of ether to remove unsaponified material. The aqueous solution was then 15 made acid to pH 1 and extracted with 150 milliliters of ether, after which the ether layer was separated and dried over anhydrous sodium sulfate. After separation from the dehydrating agent, ether was distilled off. The residue 20 from ether solution, amounting to 9.36 grams, was recrystallized from 5:1 hexane-ethyl acetate solvent and yielded white crystals melting at  $146-147^{\circ}$  C.

Potentiometric titration with 0.10 N methanolic potassium hydroxide of the sample dissolved in dimethyl 25 formamide, calculated neutralization equivalent weight for  $C_{22}H_{35}O_6NS$ , N-(n-dodecylbenzenesulfonyl) iminodiacetic acid, first end point  $-441$ ; second end point  $-220.5$ ; found, first end point  $-449$ ; found, second end point  $-219.5$ .

30 Example 3 of corrosion inhibitor—(N-dodecylbenzenesulfonyl) sarcosine technical

(A) PREPARATION OF DODECYLBENZENESULFONYL CHLORIDE

35 This compound was prepared in the following manner from a commercial grade of dodecylbenzene. One-half mole of dodecylbenzene (123 grams) was dissolved in 200 milliliters of methylene chloride in a 1-liter flask fitted with a mechanical stirrer, an air-condenser, thermometer and dropping funnel; the entire apparatus was protected from moisture by calcium chloride drying tubes on the condenser and dropping funnel. After cooling the methylene chloride solution to  $-8^{\circ}$  C. by an external bath, chlorosulfonic acid (145.5 g.) (1.2 moles) was added thereto, dropwise, over a period of one hour and fifty minutes while the temperature of the reaction mixture was maintained between  $-9$  and  $-2^{\circ}$  C. The reaction mixture became increasingly dark brown in color as the addition of chlorosulfonic acid proceeded. 40 It was stirred an additional two hours while maintaining its temperature at  $0^{\circ}$  C., whereupon it was allowed to stand at room temperature for about 16 hours. It was then poured into a mixture of 500 milliliters of 15% aqueous sodium chloride and about 300 grams of ice, and stirred well. Diethyl ether in an amount of 300 milliliters was added, and intimately mixed with the reaction mixture, whereupon after stratification the upper organic layer was separated and washed with several 75 milliliter portions of water containing 5% sodium bicarbonate and 10% sodium chloride. The ether-methylene chloride solution was dried over solid anhydrous sodium sulfate overnight, separated from the latter, after which the organic solvent mixture was removed by distillation. The residue was a dark brown liquid, insoluble 55 in water; it weighed 120 grams. The yield of crude product was therefore about 70% of theory.

60 Analysis of the crude sulfonyl chloride gave the following results:

|                                | Wt. percent |
|--------------------------------|-------------|
| Dodecylbenzenesulfonylchloride | 87.1        |
| Dodecylbenzenesulfonic acid    | 14.8        |

75 The analytical results indicated that the product as described above could be used as a reactant in this and the next example.

## (B) PREPARATION OF N-DODECYLBENZENESULFONYL SARCOSINE FROM PRODUCT (A) SUPRA

Nine and two-tenths grams (9.2 g.) (0.10 mole) of sarcosine which was 96.6% pure was dissolved in 100 milliliters of water containing 4.1 grams (0.10 mole) of sodium hydroxide. Dodecylbenzenesulfonyl chloride described in (A) above (39.2 grams) (0.10 mole) was dissolved in dioxane so that a volume of 70 milliliters was obtained. The dioxane solution of it and 70 milliliters of aqueous alkali (containing 4.7 grams of sodium hydroxide) were added simultaneously to the stirred sarcosine solution over a period of 30 minutes, the temperature of the reaction varying from 28° C. to 37° C. The reaction mixture was stirred at 45° C. for one hour and then let stand at room temperature for about sixteen hours. This contained the sodium salt of N-dodecylbenzenesulfonyl chloride sarcosine-technical. It was then made acid to pH 3 with 6 N aqueous hydrochloric acid after which it was extracted with two 200 milliliter portions of diethyl ether. The ether layer was dried over anhydrous sodium sulfate. After this dehydration step and separation from the sodium sulfate, ether was removed by distillation. The residue was an amber-like gummy mass having a neutralization equivalent of 485. The theoretical neutralization equivalent for N-(dodecylbenzenesulfonyl) sarcosine is 397. The reaction product thus has an analysis which varies quite appreciably from that expected for (N-dodecylbenzenesulfonyl) sarcosine.

*Example 4 of corrosion inhibitor.—Reaction product of technical dodecylbenzenesulfonyl chloride with iminodiacetic acid*

Iminodiacetic acid (2 g.) (0.015 mole) and triethylamine (4.55 g.) (0.045 mole) were mixed in boiling chloroform, and after cooling to room temperature the 90% dodecylbenzenesulfonyl chloride, prepared by Example 3(A) supra, in an amount of 5.15 grams (0.0105 mole) was added. The mixture was shaken vigorously for 20 minutes, then allowed to stand at room temperature overnight (about 16 hours). It was then refluxed for an hour before filtering the insoluble material. The chloroform was removed by distillation in vacuo. The residue, which represented the triethylamine salt of technical (N-dodecylbenzenesulfonyl) iminodiacetic acid, was acidified to pH 1 with aqueous 6 N hydrochloric acid after which the solution was extracted several times with ether. The ether extracts were washed with dilute hydrochloric acid and water and thereafter dried over anhydrous sodium sulfate. After decantation from the dehydrating agent, the ether was removed by distillation. The residue was an amber colored, semi-hardened mass, weighing 1.4 grams. It has a neutralization equivalent of 548. The reaction product thus has an analysis which varies quite appreciably from that expected for (N-dodecylbenzenesulfonyl) iminodiacetic acid.

*Example 5 of corrosion inhibitor.—Reaction product of dodecylbenzenesulfonyl chloride with dimethyliminodiacetate hydrochloride*

Dimethyliminodiacetate hydrochloride (20.0 grams) (0.10 mole) was dispersed in 200 milliliters of chloroform, and 24.3 grams of triethylamine (0.24 mole) was added rapidly while the chloroform dispersion was stirred. Dodecylbenzenesulfonyl chloride was dissolved in 125 milliliters of chloroform and added dropwise over a period of one hour to the stirred chloroform solution of dimethyliminodiacetate. The turbid reaction mixture was stirred at room temperature for an additional hour, then washed successively with water and 5 percent aqueous sodium chloride solution, after which the chloroform solution was dried over anhydrous sodium sulfate. After separation from the sodium sulfate the chloroform was distilled. The residue was dissolved in 300 milliliters of 50% aqueous methanol containing 17 grams of potassium hydroxide

and warmed on the steam bath for one hour with occasional stirring. The reaction solution of the potassium salt of (N-dodecylbenzenesulfonyl) iminodiacetic acid was diluted with an equal volume of water, made acid to pH 1 with 6 N aqueous hydrochloric acid and extracted with two 200 milliliter portions of ether. The ether solution of the free (N-dodecylbenzenesulfonyl) iminodiacetic acid was then dried over anhydrous sodium sulfate. After decantation from the drying agent the ether was distilled off. The residue from ether weighed 32.9 grams and had a neutralization equivalent of 415. The theoretical neutralization equivalent for (N-dodecylbenzenesulfonyl) iminodiacetic acid is 220.5 indicating that the product is a mixture of (N-dodecylbenzenesulfonyl)-iminodiacetic acid and its methyl esters.

In order to demonstrate the outstanding properties of the N-(alkylarylsulfonyl) amino acids and their salts, which are the corrosion inhibitors of the present invention, rust test data and emulsion test data were obtained for a selected mineral oil containing the respective products synthesized in Examples 1, 2, 3, 4 and 5 described above.

The oil used in these was a solvent-refined and filtered non-additive turbine-grade lubricating mineral oil of 150 Saybolt Universal Seconds viscosity at 100° F.

The rust test which was selected because it has been widely used was the "Static Water Drop Corrosion Test" developed by Zisman et al. and described in "Industrial and Engineering Chemistry," vol. 41, page 137 ff. (1949). Briefly, the test consists essentially of observing rusting at 140° F. in the presence of liquid water in the dimple of a triangular cold-rolled steel specimen immersed in the test oil. An effective rust preventive oil will prevent rusting for several days while straight mineral oils permit rusting to occur within 2 hours of test.

Solubilization of these N-(alkylarylsulfonyl) amino acids of these examples was effected by the addition of a solubilization agent which per se in oil solution had little, if any, rust preventive properties. The specific agent used was a commercially available tertiary alkyl primary amine, the tertiary alkyl groups having from 18 to 24 carbon atoms, known as "Primene JMR," which is described more exactly in a footnote in Table I.

The test used for determining the demulsibility properties of lubricating oils is to be found in the Federal Standard Stock Catalogue method 320.1.5 dated November 15, 1948, and entitled "Emulsion (Lubricating Oils)." Briefly, this test involves mixing 40 milliliters of water and 40 milliliters of test oil at 130° F. or 180° F. under standard conditions and observing the separation of oil and water phases at the test temperature. The test temperature selected is usually 130° F. for light viscosity turbine oils up to about 500 Saybolt Universal seconds viscosity at 100° F., and that was the temperature which was selected for the tests reported. The figures in the table show the number of minutes at which there is no continuous layer of emulsion between the oil and the emulsant (water). The U.S. Navy specifies that 2190-T grade turbine oils separate from water in this test within thirty minutes and have not more than 3 milliliters of an intermediate oil-and-water phase at this time in order to comply with MIL-L-17331 (Ships) Specification of September 30, 1952. This criterion of demulsibility is widely adopted by turbine oil producers and consumers.

For comparison, in order to determine quantitatively the effect of other additives to the mineral lubricating oil, both on rust prevention and imparting different emulsification characteristics, the corrosion test and the emulsion test were run on the base oil as a check, the tertiary-alkyl primary amine (2 concentrations) in the oil, stearic acid in the oil, and mixture of stearic acid with the tertiary-alkyl primary amine in the oil, as well as the oil containing the investigated N-(alkylarylsulfonyl) amino acids in the compositions given in the appended table.

The pertinent test results are set forth in Table I.

TABLE I.—RUST PREVENTIVE AND DEMULSIBILITY PROPERTIES OF (N-ALKYLARYLSULFONYL) AMINO ACIDS IN LUBRICATING OIL

| Additive (X)                                                                         | Example No. | Wt. per cent of (X) | Wt. per cent of "Primene JMR" | Emulsion Test—Time for Complete Separation (Minutes) | "Static Water Drop—Corrosion Test" Time to Rust (Hours) |
|--------------------------------------------------------------------------------------|-------------|---------------------|-------------------------------|------------------------------------------------------|---------------------------------------------------------|
| Base Oil                                                                             |             | None                | None                          | 10                                                   | Less than 16.                                           |
| "Primene JMR" <sup>1</sup>                                                           |             | None                | 0.20                          |                                                      | Do.                                                     |
| "Primene JMR"                                                                        |             | None                | 0.0125                        | 10                                                   |                                                         |
| Stearic Acid                                                                         |             | 0.20                | None                          |                                                      | Do.                                                     |
| Stearic Acid and "Primene JMR"                                                       |             | 0.20                | 0.20                          |                                                      | Less than 2.                                            |
| N-(n-dodecylbenzenesulfonyl) sarcosine                                               | I           | 0.025               | 0.025                         |                                                      | More than 300 hrs.                                      |
| N-(n-dodecylbenzenesulfonyl) iminodiacetic acid                                      | II          | 0.025               | 0.0125                        |                                                      | Do.                                                     |
| (N-dodecylbenzenesulfonyl)sarcosine (technical)                                      | III         | 0.0125              |                               | 15                                                   | Do.                                                     |
| Do                                                                                   | III         | 0.0125              |                               | 15                                                   | Do.                                                     |
| Reaction Product of technical dodecylbenzenesulfonyl chloride and iminodiacetic acid | IV          | 0.0125              | 0.0125                        | 0                                                    | Do.                                                     |
| Do                                                                                   | IV          | 0.0125              |                               | 6                                                    | Do.                                                     |
| (N-dodecylbenzenesulfonyl)iminodiacetic acid (technical)                             | V           | 0.0125              |                               | 6                                                    | Do.                                                     |
| Do                                                                                   | V           | 0.0125              | 0.0125                        | 12                                                   | Do.                                                     |

<sup>1</sup> "Primene JMR" is a mixture of branched, primary amines in which the primary amino nitrogen group is directly attached to a tertiary carbon atom, and being composed of amines from eighteen to twenty-four carbon atoms; the predominant portion may be represented by the formula  $t-C_{18-24}H_{37}-NH_2$ . It contains about 8-10% non-amine material. This trademarked product is marketed by Rohm & Haas Company of Philadelphia, Pennsylvania.

From the data set forth in this table it is apparent that a much improved rust preventive effectiveness is imparted to lubricating oil which contains the N-(alkylarylsulfonyl) amino acids of the present invention, whether the comparison is made on the base oil alone or with the solubilizer in the oil. It is also evident that the N-(alkylarylsulfonyl) amino acids are qualitatively superior in rust preventive effectiveness than a typical high molecular weight fatty acid, such as stearic acid, or the latter admixed with the identical solubilizer.

It is apparent from the emulsion test data given in the table that the alkylarylsulfonyl amino acids tested do not impart undesirable emulsion characteristics to the turbine oil.

The vehicle can be aqueous which includes aqueous solutions of liquids, such as alcohol-water mixtures, or the like. Non-limiting examples of suitable vehicles for the corrosive inhibitor additives of this invention are mineral lubricating oils of all grades; gasolines and other light petroleum products, such as fuel oil; water, alcohols, such as ethanol, isopropanol, butanol, cyclohexanol, methylcyclohexanol, octanol, decanol, dodecanol, hexadecanol, octadecanol, oleyl alcohol, benzyl alcohol, etc.; glycols, such as ethylene glycol, propylene glycol, butylene glycol; glycerol, etc.; ketones, such as acetone, methyl ethyl ketone, dipropyl ketone, cyclohexanone, etc.; keto alcohols, such as benzoin; ethers, such as diethyl ether, dipropyl ether, dichloro diethyl ether, diphenyl oxide, polyethylene glycols as diethylene glycol and triethylene glycol, ethylene glycol monobutyl ether, etc.; neutral esters, such as ethyl acetate, butyl propionate, cresyl acetate, dodecyl acetate, ethyl maleate, butyl stearate, tridecyl phosphate, tributyl trithiophosphate, triamyl phosphite, dibutyl sebacate and diethyl sebacate, etc.; petroleum waxes, such as slack wax and paraffin wax; natural waxes, such as carnauba wax, japan wax, beeswax, etc.; natural fats and oils, such as sperm oil, tallow, cottonseed oil, castor oil, linseed oil, tung oil, soybean oil, oiticica oil, tar oil, oleo oil, etc.; hydrocarbons; greases; asphalts; and chlorinated petroleum fractions, such as chlorowax.

The order of amount of corrosive inhibitor additive used in these various vehicles is like that which has been set out previously as to oleaginous vehicles.

Acidic aqueous solutions for metal pickling baths can be protected against corrosive tendencies by employing our corrosion inhibitors. Hydraulic systems can be protected against corrosion by using hydraulic fluids containing additives of the present invention. Corrosive tendencies of coolants and anti-freeze solutions or mixtures, such as those used as coolants in internal combustion engines, can be reduced by addition thereto of the alkylarylsulfonyl amino acids of our invention. Such

anti-freezes include water, water-alcohol, glycols, glycol-water, etc.

Other substances in addition to the reaction products, the corrosion inhibitors of this invention can be added to compositions contemplated herein to impart other desirable properties thereto, such as anti-oxidants, pour point depressants, V.I. improvers, etc.

Some members of this class of compounds will be preferred for specific applications while other members will be preferred for other applications where rust prevention is desired. Some members of this class of compounds are particularly applicable for turbine lubrication, because lubricant compositions containing them permit ready separation of entrained water. It is essential that water be easily separable from turbine lubricants by auxiliary oil purification equipment such as settling tanks, filters, blotter presses, centrifuges, etc., because water in addition to causing rusting accelerates oil breakdown, causes excessive foaming and facilitates the dispersion of other contaminants which accelerate oil breakdown and are injurious to the lubricating system in other ways.

Although the present invention has been described with preferred embodiments, it is to be understood that modifications may be made without departing from the spirit and scope thereof, as those skilled will readily understand. Such variations and modifications are considered to be within the purview and scope of the appended claims.

We claim as our invention:

1. A corrosion-inhibiting composition which comprises a liquid vehicle which tends to permit the corrosion of metal in the service to which said vehicle is put, containing a member selected from the group consisting of N-(n-dodecylbenzenesulfonyl) sarcosine and N-(n-dodecylbenzenesulfonyl) iminoacetic acid, said member being present in said liquid vehicle in amounts of as little as a fraction of 1% by weight but in a sufficient quantity to inhibit corrosion of said vehicle.

2. A corrosion-inhibiting composition which comprises a liquid vehicle which tends to permit the corrosion of metal in the service to which said vehicle is put, containing N-(n-dodecylbenzenesulfonyl) sarcosine, said latter component being present in said liquid vehicle in amounts of as little as a fraction of 1% by weight but in a sufficient quantity to inhibit corrosion of said metal.

3. A corrosion inhibiting composition which comprises a liquid vehicle which tends to permit the corrosion of metal in the service to which said vehicle is put, containing N-(n-dodecylbenzenesulfonyl) iminodiacetic acid, said latter component being present in said liquid vehicle in amounts of as little as a fraction of 1% by weight but in a sufficient quantity to inhibit corrosion of said metal.

4. A rust-inhibited oleaginous composition adapted for

use in the presence of water in systems containing metal susceptible to corrosion by said water, comprising an oleaginous vehicle and a member selected from the group consisting of N-(n-dodecylbenzenesulfonyl) sarcosine and N-(n-dodecylbenzenesulfonyl) iminoacetic acid, said member being present in said oleaginous vehicle in amounts of as little as a fraction of 1% by weight but in a sufficient quantity to inhibit corrosion of said vehicle.

5. A rust-inhibited oleaginous composition adapted for use in the presence of water in systems containing metal susceptible to corrosion by said water comprising an oleaginous vehicle and N-(n-dodecylbenzenesulfonyl) sarcosine, said latter component being present in said oleaginous vehicle in amounts of as little as a fraction of 1% by weight but in a sufficient quantity to inhibit corrosion of said metal.

6. A rust-inhibited oleaginous composition adapted for use in the presence of water in systems containing metal susceptible to corrosion by said water comprising an oleaginous vehicle and N-(n-dodecylbenzenesulfonyl) iminodiacetic acid, said latter component being present in said oleaginous vehicle in amounts of as little as a fraction of 1% by weight but in a sufficient quantity to inhibit corrosion of said metal.

7. A rust-inhibited oleaginous composition adapted for use in the presence of water in systems containing metal susceptible to corrosion by said water, comprising an oleaginous vehicle, a member selected from the group consisting of N-(n-dodecylbenzenesulfonyl) sarcosine and N-(n-dodecylbenzenesulfonyl) iminoacetic acid in amounts of as little as a fraction of 1% but in sufficient quantity to inhibit corrosion of said metal, and an alkyl primary amine having 18-24 carbon atoms in sufficient amount to solubilize said member in the oleaginous vehicle.

8. A rust-inhibited oleaginous composition adapted for use in the presence of water in systems containing metal susceptible to corrosion by said water, comprising an oleaginous vehicle, N-(n-dodecylbenzenesulfonyl) sarcosine in amounts of as little as a fraction of 1% but in sufficient quantity to inhibit corrosion of said metal, and an alkyl primary amine having 18-24 carbon atoms in sufficient amount to solubilize said N-(n-dodecylbenzenesulfonyl) sarcosine in the oleaginous vehicle.

9. A rust-inhibited oleaginous composition adapted for use in the presence of water in systems containing metal susceptible to corrosion by said water, comprising an oleaginous vehicle, N-(n-dodecylbenzenesulfonyl) iminodiacetic acid in amounts of as little as a fraction of 1% but in sufficient quantity to inhibit corrosion of said

metal, and an alkyl primary amine having 18-24 carbon atoms in sufficient amount to solubilize said N-(n-dodecylbenzenesulfonyl) iminodiacetic acid.

10. A rust-inhibited oleaginous composition adapted for use in the presence of water in systems containing metal susceptible to corrosion by said water, comprising an oleaginous vehicle, a member selected from the group consisting of N-(n-dodecylbenzenesulfonyl) sarcosine and N-(n-dodecylbenzenesulfonyl) iminoacetic acid in amounts between substantially 0.005% to about 10% by weight, and an alkyl primary amine having 18-24 carbon atoms in sufficient amount to solubilize said member in the oleaginous vehicle.

11. A rust-inhibited oleaginous composition adapted for use in the presence of water in systems containing metal susceptible to corrosion by said water, comprising an oleaginous vehicle, N-(n-dodecylbenzenesulfonyl) sarcosine in amounts between substantially 0.005% to about 10% by weight, and an alkyl primary amine having 18-24 carbon atoms in sufficient amount to solubilize said N-(n-dodecylbenzenesulfonyl) sarcosine in the oleaginous vehicle.

12. A rust-inhibited oleaginous composition adapted for use in the presence of water in systems containing metal susceptible to corrosion by said water, comprising an oleaginous vehicle, N-(n-dodecylbenzenesulfonyl) iminodiacetic acid in amounts between substantially 0.005% to about 10% by weight, and an alkyl primary amine having 18-24 carbon atoms in sufficient amount to solubilize said N-(n-dodecylbenzenesulfonyl) iminodiacetic acid.

#### References Cited in the file of this patent

##### UNITED STATES PATENTS

|    |           |                |               |
|----|-----------|----------------|---------------|
| 35 | 2,142,847 | Hultquist      | Jan. 3, 1939  |
|    | 2,225,960 | Orthner et al. | Dec. 24, 1940 |
|    | 2,578,725 | Michel et al.  | Dec. 18, 1951 |
|    | 2,602,760 | Michel et al.  | July 8, 1952  |
| 40 | 2,656,381 | Sprague        | Oct. 20, 1953 |
|    | 2,660,562 | Axe et al.     | Nov. 24, 1953 |
|    | 2,692,857 | Michel et al.  | Oct. 26, 1954 |
|    | 2,694,045 | Jones et al.   | Nov. 9, 1954  |
|    | 2,704,264 | Michel et al.  | Mar. 15, 1955 |

##### FOREIGN PATENTS

|    |         |         |               |
|----|---------|---------|---------------|
| 45 | 900,041 | Germany | Dec. 17, 1953 |
|----|---------|---------|---------------|

##### OTHER REFERENCES

50 Tertiary-alkyl Primary Amines, Rohm & Haas, September 1954, pp. 16 and 17.